# EUROPEAN PATENT SPECIFICATION

(11) **EP 1 714 717 B1**
(45) Date of publication and mention of the grant of the patent: **02.04.2008**
(21) Application number: 06008110.6
(22) Date of filing: 19.04.2006
(51) Int. Cl.: B21J 13/02, B22C 9/06

(54) **Method of predicting damage of dies**
Verfahren zur Vorhersage des Versagens von Matrizen
Méthode de prédiction de la défaillance des matrices

(30) Priority: 19.04.2005 JP 2005120660
(43) Date of publication of application: 25.10.2006
(73) Proprietor: Daido Steel Co.,Ltd., Higashi-ku Nagoya Aichi 461-0005 (JP)
(72) Inventor: Yoshida, Hiroaki, c/o Daido Steel Co., Ltd., Minami-ku Nagoya Aichi (JP); Itoh, Shigekazu, c/o Daido Steel Co., Ltd., Minami-ku Nagoya Aichi (JP)
(74) Representative: Rupprecht, Kay

(56) References cited:
- PATENT ABSTRACTS OF JAPAN vol. 2003, no. 03, 5 May 2003 (2003-05-05) -& JP 2002 321032 A (TOYOTA MOTOR CORP; TOYOTA CENTRAL RES & DEV LAB INC), 5 November 2002 (2002-11-05)
- PATENT ABSTRACTS OF JAPAN vol. 2000, no. 12, 3 January 2001 (2001-01-03) -& JP 2000 246394 A (HITACHI METALS LTD), 12 September 2000 (2000-09-12)
- PATENT ABSTRACTS OF JAPAN vol. 2002, no. 05, 3 May 2002 (2002-05-03) -& JP 2002 001475 A (TOYOTA MOTOR CORP), 8 January 2002 (2002-01-08)
- KIM ET AL: "Estimation of die service life against plastic deformation and wear during hot forging processes" JOURNAL OF MATERIALS PROCESSING TECHNOLOGY, ELSEVIER, AMSTERDAM, NL, vol. 166, no. 3, 20 August 2005 (2005-08-20), pages 372-380, XP005023923 ISSN: 0924-0136

## Description

### BACKGROUND OF THE INVENTION

### Technical Field

The present invention concerns a method of predicting damages of dies. More specifically, the invention concerns predicting damages in dies for plastic processing of metals, typically, forging dies by predicting "great crack" damage caused by brittle fracture which dominates die lives, and utilizing the results for die design including choice of materials, hardness thereof and determining the die configuration so as to establish countermeasures for prolongation of die lives.

### Prior Art

At manufacturing and application of forging dies various methods of predicting damages in dies have been developed and utilized for enabling manufacture of dies of longer lives. As the method of prediction it is generally employed to calculate temperature and stress distribution in a die by finite element analysis and then substitute the calculated values for constitutive equations to predict low cycle fatigue lives and abrasion. For example, Japanese Patent Disclosure No. 2002-321032 discloses technique of predicting die lives on the basis of die abrasion according to an abrasion model adopting conditions inherent in forging dies.

Fracture factors causing damage of forging dies during using are four, namely, "great crack" or static brittle fracture, plastic flow, abrasion and low cycle fatigue destruction. The brittle fracture is a sudden phenomenon occurring at an initial stage before substantial use of the die, and also called "initial crack", which is a fatal damage. However, methods of predicting damage of dies proposed so far are not effective for this kind of brittle fracture. As to ductile fracture there has been proposed Cockroft's formula, Oyane's formula and Ayada's formula, which have been acknowledged. These formulae are, however, not applicable to the brittle fracture. Thus, there has been demand for formula or formulae which enable effective prediction of damage of dies caused by brittle fracture.

### SUMMARY OF THE INVENTION

The object of the present invention is to provide a method of predicting damage of dies enabling design of improved dies by predicting brittle fracture which give, among various factors causing damage to forging die, fatal influence to die lives.

The method according to the invention achieving the above-mentioned object is a method of predicting "great crack" by brittle fracture which dominates the lives of dies for plastic processing of metals to contribute to die design including choice of materials, hardness and configuration of the die. The method of predicting damages of dies according to the invention is characterized in that the die design is carried out by choosing the condition that none of the predicted values of brittle fracture, F_{c1} to F_{c3}, calculated by the formulae 1 to 3 below exceed the critical values determined on the basis of the material used. ${F}_{c ⁢ 1} = \left({σ}_{m}/{σ}_{eq}\right)$ ${F}_{c ⁢ 2} = \left({σ}_{m}/{σ}_{1 ⁢ max}\right)$ ${F}_{c ⁢ 3} = \left({σ}_{1 ⁢ max}/{σ}_{eq}\right)$
σₘ: mean normal stress loaded to the tensile side of the
   die
σ_{eq}: Von Misese's equivalent stress
σ₁ₘₐₓ: maximum principal stress

### BRIEF EXPLANATIO OF THE DRAWINGS

Fig. 1 is a plan view illustrating the shape and dimension of a smooth test piece of the tensile test pieces prepared for constructing database of the material properties prior to conducting the present invention;
Fig. 2 is a plan view like Fig. 1 illustrating the shape and dimension of the test piece having a surrounding V-notch with notch angle of 30°;
Fig. 3 is a plan view like a part of Fig. 2 illustrating the detail of the notched part of the test piece with notch angle of 90°;
Fig. 4 is a plan view like a part of Fig. 3 illustrating the detail of the notched part of the test piece with notch angle of 120°;
Fig. 5 is a graph obtained by plotting mean normal stress (σₘ) corresponding to equivalent stress (σ_{eq}) based on the data given by tensile tests in working example of the present invention;
Fig. 6 is a graph obtained by plotting mean normal stress (σₘ) corresponding to maximum principal stress (σ₁ₘₐₓ) based on the data given by tensile tests in working example of the present invention;
Fig. 7 is a graph obtained by plotting maximum principal stress (σ₁ₘₐₓ) corresponding to equivalent stress (σ_{eq}) based on the data given by tensile tests in working example of the present invention;
Fig. 8 is a section view illustrating the shape of a ring-die and a work used at hot forging a final gear (an automobile part);
Fig. 9 is data of a working example and a computer graphics (hereinafter referred to as "CG") obtained by FEM analysis showing distribution of the critical values F_{c1} of brittle fracture in a ring-die before improvement by the invention;
Fig 10 is a CG like Fig. 9 showing distribution of the critical values F_{c2} of brittle fracture in a ring-die before improvement by the invention;
Fig 11 is a CG like Fig. 9 showing distribution of the critical values F_{c3} of brittle fracture in a ring-die before improvement by the invention;
Fig 12 is a CG like Fig. 9 showing distribution of the critical values F_{c1} of brittle fracture in a ring-die after improvement by the invention;
Fig 13 is a CG like Fig. 9 showing distribution of the critical values F_{c2} of brittle fracture in a ring-die before improvement by the invention;
Fig 14 is a CG like Fig. 9 showing distribution of the critical values F_{c3} of brittle fracture in a ring-die before improvement by the invention;

### DETAILED EXPLANATION OF THE PREFERRED EMBODIMENTS

The factors dominating the brittle fracture of dies are three, as noted above, i.e., mean normal stress (σₘ), equivalent stress (σ_{eq}) and maximum principal stress (σ₁ₘₐₓ). It can be hence said that there is generally the following relation: $F ⁢ c = f \left({σ}_{m}, ⁢, {σ}_{eq}, ⁢, {σ}_{1 ⁢ max}\right)$

All the dominating factors are considered in the above formulae 1 to 3. In practical use of these formulae an improved formula or formulae (such as those with adjusted coefficients) may be found by experience. They will give the same effect as those discussed above, and thus the invention includes the embodiments using such formulae.

By predicting the damages of dies it will be possible to establish effective countermeasures to the brittle fracture (so-called "great crack" or "initial crack"), to which, though it is an important factor, no conventional method of predicting damages has not been confronted. Those skilled in the art will be able to manufacture the optimum die by constructing databases in regard to the respective steels with reference to the working examples described below, by choosing the condition where all the predicted brittle fracture values F_{c1} to F_{c3} do not reach the critical limits, and by designing the dies. If the dies enjoy prolonged lives it will contribute to decrease in processing costs of various forged products through not only reducing the die cost itself but also saving time and labor for exchanging the worn dies.

The method of predicting damages of dies according to the invention may exhibit the performance to the dies for forming. It will be, however, applicable to other dies such as those for die-casting, which are used under similar environment of high temperature and high stress. Through the prediction of damages of dies desired properties of die materials may be known as a matter of course and the indices for developing the die materials can be obtained. Thus, the invention may contribute to development of alloy technologies.

### EXAMPLES

### Example 1

SKD61, one of the steels for hot processing tools, was used as the die material and the hardness was adjusted to be HRC 46, 49 or 52. JIS No.4 tensile test pieces were prepared and some of them were subjected to machining to provide surrounding V-shaped notches of depth 50%. The shapes and dimensions of the test pieces are shown in Fig. 1 (smooth surface), Fig. 2 (notch angle 30°), Fig. 3 (90°) and Fig. 4 (120°). Curvature of the bottom of the notches is 0.2mm.

The test pieces were subjected to tensile tests to determine mean normal stress (σₘ) at which fracture occurs and at the same time whether the fracture is ductile fracture or brittle fracture was recorded. The equivalent stress (σ_{eq}) and the maximum principal stress (σ₁ₘₐₓ) were calculated. By plotting the mean normal stress (σₘ) in correspondence of the equivalent stress (σ_{eq}) there was obtained Fig. 5, by plotting the mean normal stress (σₘ) in correspondence of the maximum principal stress (σ₁ₘₐₓ), Fig. 6, and plotting the maximum principal stress (σ₁ₘₐₓ) in correspondence of the equivalent stress (σ_{eq}), Fig. 7, respectively.

Based on the graphs of Figs. 5 to 7 the critical values C₁ to C₃ for the brittle fracture of SKD61 steel were determined as follows: ${F}_{c ⁢ 1} = \left({σ}_{m}/{σ}_{eq}\right) = 0.7$ ${F}_{c ⁢ 2} = \left({σ}_{m}/{σ}_{1 ⁢ max}\right) = 0.5$ ${F}_{c ⁢ 3} = \left({s}_{1 ⁢ max}/{s}_{eq}\right) = 1.25$

### Example 2

The prediction of die life according to the present invention was carried out in regard to a ring-die, a die for limiting the outer surface of the work forged by a punch and a counter punch from top and bottom used for hot forging a final gear, an automobile part, having the cross section shown in Fig. 8. A used die made of SKD61 steel was inspected and it was found that crack of the ring-die occurred from the outer surface.

The following three CG's were obtained by analyzing distribution of the critical fracture values F_{c1} to F_{c3} on the basis of the above database by computer simulation (FEM analysis). $\left(former shape\right) {F}_{c ⁢ 1} = \left({σ}_{m}/{σ}_{eq}\right)$ $\left(former shape\right) {F}_{c ⁢ 2} = \left({σ}_{m}/{σ}_{1 ⁢ max}\right)$ $\left(former shape\right) {F}_{c ⁢ 3} = \left({σ}_{1 ⁢ max}/{σ}_{eq}\right)$

All the CG's showed that in some parts of outer surface of the ring-die F_{c1} to F_{c3} exceed the critical values. The fact agrees with the results of the above inspection.

Then, supposing the cases where the outer diameter of the ring-die is increased to prevent the brittle fracture, the computer simulation was carried out again. Three CG's as mentioned below were obtained. The CG's showed that there existed no longer the parts where the F_{c1} to F_{c1} exceeded the critical values. $\left(improved shape\right) {F}_{c ⁢ 1} = \left({σ}_{m}/{σ}_{eq}\right)$ $\left(improved shape\right) {F}_{c ⁢ 2} = \left({σ}_{m}/{σ}_{1 ⁢ max}\right)$ $\left(improved shape\right) {F}_{c ⁢ 3} = \left({σ}_{1 ⁢ max}/{σ}_{eq}\right)$

## Claims

1. A method of predicting damage of dies used for plastic processing of metallic materials by predicting "great crack" caused by brittle fracture dominating the die lives so as to contribute to die design including choice of die materials, hardness of the material and determination of die shape, which comprises carrying out the die design by selecting the conditions that none of the anticipated brittle fracture values F_{c1} to F_{c3} calculated by the formulae below exceed the critical values depending on the materials: ${F}_{c ⁢ 1} = \left({σ}_{m}/{σ}_{eq}\right)$ ${F}_{c ⁢ 2} = \left({σ}_{m}/{σ}_{1 ⁢ max}\right)$ ${F}_{c ⁢ 3} = \left({δ}_{1 ⁢ max}/{δ}_{eq}\right)$
where,
σₘ: mean normal stress loaded to the tensile side of the die;
σ_{eq} : Von Misese's equivalent stress ;
σ₁ₘₐₓ : maximum principal stress.

2. The method of predicting damage of die according to claim 1, wherein the material of the die is SKD61 steel and F_{c1}=0.7, F_{c2}=0.5 and F_{c3}=1.25.

## Patentansprüche

1. Verfahren zur Vorhersage von Schäden in Matrizen, die zur plastischen Bearbeitung von metallischen Materialien verwendet werden, durch die Vorhersage des Gewaltbruchs, der durch den die Lebensdauer von Matrizen bestimmenden Sprödbruch verursacht wird, um zur Auslegung und Konstruktion der Matrize einschließlich der Wahl der Matrizenmaterialien Materialien, der Härte des Materials und der Bestimmung der Matrizenform beizutragen, das die Ausführung der Auslegung der Matrize aufweist, indem die Bedingungen gewählt werden, bei denen keiner der vorhergesagten Werte des Sprödbruchs, F_{c1}, bis F_{c3}, die mit den nachstehenden Formeln 1 bis 3 berechnet werden, die materialabhängigen kritischen Werte überschreitet: ${F}_{c ⁢ 1} = \left({σ}_{m}/{σ}_{eq}\right)$ ${F}_{c ⁢ 2} = \left({σ}_{m}/{σ}_{1 ⁢ max}\right)$ ${F}_{c ⁢ 3} = \left({σ}_{1 ⁢ max}/{σ}_{eq}\right) ;$
dabei:
σₘ: mittlere Normalspannung, die die Zugseite der Matrize belastet;
σ_{eq}: von Misese'sche äquivalente Spannung;
σ₁ₘₐₓ: maximale Hauptspannung.

2. Verfahren zur Vorhersage von Schäden in Matrizen nach Anspruch 1, bei dem das Material der Matrize SKD61-Stahl ist und F_{c1} = 0,7; F_{c2} = 0,5 und F_{c3} = 1,25.

## Revendications

1. Procédé pour prédire une détérioration de matrices utilisées pour une transformation plastique de matériaux métalliques en prédisant une "fissure importante" causée par une rupture fragile dominante pendant les vies des matrices de manière à contribuer à la conception des matrices incluant le choix des matériaux de matrice, la dureté du matériau et la détermination de la forme de matrice, qui comporte la mise en oeuvre de la conception de la matrice en sélectionnant les conditions qu'aucune des valeurs de rupture fragile anticipées F_{c1} à F_{c3} calculées par les formules ci-dessous ne dépasse les valeurs critiques en fonction des matériaux : ${F}_{c ⁢ 1} = \left({σ}_{m}/{σ}_{eq}\right)$ ${F}_{c ⁢ 2} = \left({σ}_{m}/{σ}_{1 ⁢ max}\right)$ ${F}_{c ⁢ 3} = \left({σ}_{1 ⁢ max}/{σ}_{eq}\right)$
où,
σₘ est la contrainte normale moyenne appliquée du côté traction de la matrice,
σ_{eq} est la contrainte équivalente de Von Misese,
σ₁ₘₐₓ est la contrainte principale maximale.

2. Procédé pour prédire une détérioration de matrice selon la revendication 1, dans lequel le matériau de la matrice est de l'acier SKD61 et F_{c1} = 0,7, F_{c2} = 0,5 et F_{c3} = 1,25.
